

Patented Jan. 31, 1939

2,145,792

# UNITED STATES PATENT OFFICE

2,145,792

## CONTACTING ELEMENT

Franz R. Hensel and Earl I. Larsen, Indianapolis,  
Ind., assignors to P. R. Mallory & Co., Inc.,  
Indianapolis, Ind., a corporation of Delaware

No Drawing. Application March 22, 1937,  
Serial No. 132,296

5 Claims. (Cl. 200—166)

This invention relates to electric contacting elements.

An object of the invention is to improve electric contacting elements of the types including contactor contacts, circuit making and breaking contacts, switch contacts, commutator contacts, sliding contacts, trolleys, trolley shoes and the like.

Other objects of the invention will be apparent from the following description taken in connection with the appended claims.

The present invention comprises the combination of elements, methods of manufacture, and the product thereof brought out and exemplified in the disclosure hereinafter set forth, the scope of the invention being indicated in the appended claims.

While a preferred embodiment of the invention is described herein, it is contemplated that considerable variation may be made in the method 20 of procedure and the combination of elements without departing from the spirit of the invention.

A feature of the present invention is the provision of an electric contact member of a composition which has a high current carrying capacity and is resistant to mechanical wear. Other advantages are a low contact resistance which remains uniform throughout the life of the contact.

30 In one of its aspects the invention makes possible the manufacture of contacts having the desirable properties mentioned by casting, such as die or sand casting. It is found that contacts of the composition contemplated can possess high hardness in the "as cast" condition.

The contacts of the present invention also lend themselves to further hardening by heat treatment.

According to the present invention the contacts are composed predominantly of copper with addition of cobalt and cadmium. In some instances it may be desirable to add small proportions of other ingredients to the composition. For example, it has been found that heat treatment can be made more effective by the addition of small quantities of one or more of the elements silicon, beryllium or phosphorus.

The contacts may be formed of an alloy of the following composition:

### Permissible range

Per cent  
.1 to 10  
.1 to 10  
Balance

Cobalt  
Cadmium  
Copper

### Preferred range

|         | Per cent  |
|---------|-----------|
| Cobalt  | 1 to 5    |
| Cadmium | .75 to 4  |
| Copper  | Balance 5 |

The age-hardening and physical properties of the contacts may be improved by the addition of .01 to 5% of silicon, phosphorus or beryllium although the preferred proportions of these ingredients is within the range .01 to 2%. It is also understood that small proportions of other materials which do not deleteriously affect the properties may be present.

The alloy for making the contacts may be formed by melting together the proper proportions of the ingredients. It has been found of advantage to add the cobalt and cadmium to a copper melt in the form of a mixture of powders of copper, cobalt and cadmium. These powders may all be mixed together or the cobalt and cadmium powder may be mixed separately with copper powder.

It has been found of advantage in certain cases where high percentages of cadmium are required in the contact to manufacture the contacts by starting out with a powder mixture of copper, cobalt and cadmium, compressing same and sintering after compressing at a temperature high enough to secure alloying but low enough to avoid the evaporation of the cadmium. Due to the low melting point of cadmium the formation of an alloy by this method can be readily accomplished. It will also be possible to add silicon or phosphorus to such mixtures employed for sintering. The material can be used for contactor contacts in the "as sintered" condition, or a special heat treatment mentioned below can be applied after sintering.

If the alloy is produced by melting and not by sintering the contacts, may, if desired, be cast directly into the desired shape.

After casting the contacts have a hardness of 70 to 90 Rockwell B according to composition. They may be subjected to a heat treatment which may comprise heating to a high temperature, preferably in the order of 900° C., quenching, and then ageing at a lower temperature such as at about 450° C. In most instances it is possible to eliminate the quenching operation and use the low temperature treatment only to improve the thermal and electrical conductivities.

It is also possible with the composition described to deposit the material on a copper, copper alloy or similar metal plate by means of gas 55

welding or electric arc welding and then heat treating the deposit in the manner described to provide a hardened contact.

Whereas copper oxidizes readily, thereby forming a high resistance contact surface, the present composition is resistant to oxidation, maintaining a uniformly high conductivity contact surface over long periods of service. Contacts of pure copper and contactors made according to this invention were tested for increase in contact resistance by operation in a 60 cycle, 550 volt A. C. circuit carrying 100 amperes. The load used consisted of air core reactors and resistance grids in series. The contactors were operated 30 times per minute in this circuit.

After 500,000 operations the pure copper contactors increased in resistance to 1.60 milliohms. Cast contacts of the composition:

|           | Per cent   |
|-----------|------------|
| 20 Cobalt | 2.4 to 2.5 |
| Cadmium   | 2.0        |
| Silicon   | .6         |
| Copper    | Balance    |

actually decreased in resistance from about .25 milliohm at the start of the test to about .16 milliohm after 500,000 operations.

|           | Per cent |
|-----------|----------|
| 30 Cobalt | 2.5      |
| Cadmium   | 2.0      |
| Beryllium | .4       |
| Copper    | Balance  |

had a contact resistance of .43 milliohm after the same operation.

This indicates the improvement in contact

resistance of contacts of the present invention. As already indicated the other characteristics are also improved. It is likewise apparent that by a heat treatment the contacts can be age hardened whereby their strength and wear resistance is greatly enhanced.

While the present invention, as to its objects and advantages, has been described herein as carried out in specific embodiments thereof, it is not desired to be limited thereby but it is intended to cover the invention broadly within the spirit and scope of the appended claims.

What is claimed is:

1. An electric contacting element composed of about .1 to 10% cobalt, about .1 to 10% cadmium and the balance substantially all copper. 15

2. An electric contacting element according to claim 1 containing from .01 to 5% of an element selected from the group consisting of silicon, phosphorus and beryllium. 20

3. An electric contacting element according to claim 1 containing from .01 to 2% of an element selected from the group consisting of silicon, phosphorus and beryllium.

4. An electric contacting element composed of about .1 to 10% cobalt, .1 to 10% cadmium, .01 to 2% silicon and the balance substantially all copper. 25

5. An electric contacting element comprising a sintered metal product composed of about .1 to 10% cobalt, about .1 to 10% cadmium, .01 to 5% of an element selected from the group consisting of silicon and phosphorus and the balance, substantially all copper. 30

FRANZ R. HENSEL.  
EARL I. LARSEN. 35